

Feb. 7, 1928.

1,658,062

W. A. SPRAGUE

CARNAUBA WAX AND THE PREPARATION THEREOF

Filed March 15, 1926

Fig.1.



Fig.2.



Fig.3.



Fig.4.



Fig.5.



Fig.6.



INVENTOR-

William A. Sprague  
By his Attorney,  
Nelson W. Howard

## UNITED STATES PATENT OFFICE.

WILLIAM A. SPRAGUE, OF ISLINGTON, MASSACHUSETTS, ASSIGNOR TO UNITED SHOE MACHINERY CORPORATION, OF PATERSON, NEW JERSEY, A CORPORATION OF NEW JERSEY.

## CARNAUBA WAX AND THE PREPARATION THEREOF.

Application filed March 15, 1926. Serial No. 94,868.

This invention relates to the preparation of carnauba wax in the form of coherent cakes and to such coherent cakes. Carnauba wax is a secretion obtained from the buds and leaves of the Brazilian wax palm (*Copernicia cerifera*). The leaves from which the wax is obtained are dried and beaten and the resultant dust gathered up and melted. When the wax cools, it cracks into irregular pieces, the greater portion of the wax being in pieces from the size of a hen's egg or a little larger down to a fine powder, with occasional larger lumps ranging up to half a pound or more in weight. Prior to the present invention, this was the only form in which pure or unadulterated carnauba wax was known. In this form it is sacked and shipped from Brazil. As the wax is brittle, there is a continuous tendency for the larger pieces to break up and for the amount of powder to increase.

Among the different uses of carnauba wax is the polishing of various articles, for example, lasts and shoes, to which the wax is applied by means of rotary brushes or pads. The small pieces of wax and the dust are useless for such purposes, since the wax is applied to the brushes or pads by holding pieces of it against them by hand as they rotate. Thus, carnauba wax has heretofore been sorted by the importers or dealers, only the larger pieces of wax being sold for the purposes just referred to. Such selection of course considerably increased the cost of the wax to the purchaser. The selected wax, moreover, after it has been sorted, continues to break down under the treatment it receives during shipment to the consumer, so that, even after buying the selected grade, the shoe or last manufacturer accumulates quantities of carnauba wax in the form of small pieces or dust which he is unable to utilize and which must be wasted or disposed of at a loss.

Attempts have been made in the past to cast carnauba wax into uniform cakes but such attempts prior to the present invention have been uniformly unsuccessful, since it was found that upon cooling the cakes cracked and broke to pieces. This condition was so well understood in the trade that it was generally regarded as impossible to cast unadulterated carnauba wax into coherent cakes. It was recognized, however, that if the carnauba wax were mixed with certain

other materials it could be prepared in such form; but these materials (for example, paraffin) softened the wax and, accordingly, detracted greatly from its value as polishing material for such articles as shoes and lasts where a hard finish is desirable.

After a long series of experiments, I have worked out a method of preparing pure carnauba wax in the form of fine-grained coherent cakes having sufficient strength to stand up without breakage under the conditions normally incident to the handling of the wax both in shipment and in its application to the rotary brushes and pads of polishing machines. In carrying out this novel method, the wax is melted at a temperature low enough to prevent it from becoming burned. It is then preferably allowed to stand and settle, and then is cast in hot molds which are caused to cool very slowly, the cooling, from a temperature slightly above the melting point of the wax (about 216° Fahrenheit) to the room temperature, taking place in from twelve to twenty-four hours, or longer, according to the sizes of the cakes which are being cast.

In another aspect, the invention comprises, as a new article, pure or unadulterated carnauba wax in the form of coherent cakes.

The invention will now be described with reference to the accompanying drawings which illustrate diagrammatically the herein described new method of preparing carnauba wax in cake form.

In the drawings:—

Fig. 1 represents a typical sample of carnauba wax in the condition in which it is imported into this country;

Fig. 2 illustrates the melting of the wax in a covered receptacle;

Fig. 3 illustrates the wax standing in the covered receptacle without the application of heat after it has been melted;

Fig. 4 illustrates the casting of the wax in a hot mold;

Fig. 5 illustrates the slow cooling of the wax in the mold; and

Fig. 6 shows one of the smooth coherent cakes of carnauba wax thus prepared.

In the drawings the order of succession of the various steps in the preparation of applicant's new product is indicated by the arrows connecting the different figures, as well as by the numbers of the figures themselves.

Fig. 1 represents a sample of carnauba wax of the grade known commercially as No. 1 yellow. It is of a light yellow color and consists of pieces varying in size from a hen's egg or a little bigger down to dust, with the greater portion of the wax in pieces from the size of English walnuts down to dust. While this is a good grade of wax, being the second out of six recognized commercial 10 grades, it contains an appreciable quantity of dirt. This, however, is inconspicuous and for the most part invisible.

The preparation of the wax will be described herein with reference to a batch of 15 about fifty pounds, since such a batch constitutes a convenient working unit. The batch of wax is placed in a covered receptacle as indicated at 10 in Fig. 2, and is heated, for example, by an electric heating 20 unit 12. During the melting the temperature of the wax must be kept below its burning point. It should not be permitted to rise above 220° Fahrenheit. On the other hand, at least with batches of this size, it 25 appears to be impractical to keep the temperature much below 216° Fahrenheit, and the latter figure may be accepted as good practice. During the melting of the wax, which will take about an hour and a half 30 or two hours, a light colored, nearly white scum consisting of foamy material illustrated at 14 with crust-like portions illustrated at 16 forms upon the top of the darker colored molten wax 18 (Fig. 2). 35 After the wax is melted, the heat is turned off and the wax in the covered receptacle is allowed to stand for about twenty minutes, as indicated in Fig. 3. During this time, the scum 14, 16 is for the most part redissolved, leaving the top of the wax substantially clear, as indicated at 20. Also, what ever dirt or other impurities are present settle to the bottom of the receptacle. The wax is then removed, leaving the settling 40 which contain the dirt in the bottom of the receptacle, and is poured into sheet metal molds 22 (Fig. 4) which have been previously heated to a temperature about that of the molten wax. The molds of hot wax 45 are then protected from rapid cooling, for example by suitable heat-insulating material indicated at 24 (Fig. 5), the cooling being controlled so that it takes from about twelve hours, in the case of small cakes of about 50 one-quarter of a pound each, up to twenty-four hours for cakes weighing one and a half or two pounds, still slower cooling being necessary if the cakes are much larger than that. When the cakes of wax are thus 55 cooled, the formation of internal stresses sufficient to cause the cakes to crack or break is avoided. Moreover, the wax shrinks as it cools sufficiently so that the cakes loosen themselves from the molds and can be re- 60 moved readily.

The cakes of carnauba wax thus prepared are attractive in appearance, are smooth, and of a color which the trade recognizes as better than that of the raw carnauba wax from which they were prepared. If one of the 70 cakes is broken, for example by a sharp blow with a hammer, its fracture is fine-grained. When casting cakes of carnauba wax by the method herein disclosed the cakes may be cast with a trademark, lettering or 75 the like, as indicated at 26 in Fig. 6, by suitably forming the bottom or other surface of the mold. This adds to the attractiveness of the cake of wax and is desirable from the merchandising point of view. 80 These cakes appear as shown in Fig. 6 and are sufficiently strong to stand handling and shipment without breakage. Thus there is substantially no waste when using the cakes for polishing purposes since each cake can 85 be used until it is too small to be held by hand against a rotary brush or pad.

While all of the herein described steps of applicant's novel method are of assistance in obtaining the best results, nevertheless 90 useful results may be obtained if certain of the steps are omitted. For example, if the molten wax is poured into cold sheet metal molds, cakes which are probably merchantable though of inferior appearance and strength will be obtained. The exterior surface of such cakes of carnauba wax, instead of being continuous and smooth, will be rough and marked with creases and cracks 95. Also, such a cake is less strong than one cast in a hot mold and upon being broken it is found that its central portion, at least, is of a much coarser structure.

Having described the invention, what I claim as new and desire to secure by Letters 105 Patent of the United States is:

1. A method of preparing coherent fine-grained cakes of unadulterated carnauba wax characterized by cooling molten carnauba wax sufficiently slowly to prevent the occurrence of internal stresses of such magnitude as to cause the cakes of wax to crack or break.

2. A method of preparing carnauba wax which comprises melting the carnauba wax 115 at a temperature insufficient to cause it to burn, pouring the molten wax into molds, and cooling the wax in the molds sufficiently slowly to prevent the occurrence of internal stresses of such magnitude as to cause the 120 cakes of wax to crack or break.

3. A method of preparing carnauba wax which comprises melting the carnauba wax at a temperature insufficient to cause it to burn, pouring the molten wax into hot molds, and cooling the wax in the molds sufficiently 125 slowly to prevent the occurrence of internal stresses of such magnitude as to cause the cakes of wax to crack or break.

4. A method of preparing smooth, co- 130

herent, fine-grained cakes of carnauba wax which comprises melting raw carnauba wax without permitting the temperature of the wax to rise sufficiently above its melting point to darken the color of the wax, removing from the molten wax any dirt that may be present, pouring the wax into hot molds, and causing the wax to cool to room temperature sufficiently slowly to prevent cracking of the cakes of wax.

5. A method of preparing carnauba wax which comprises heating raw carnauba wax in a covered receptacle and thereby melting the wax at a temperature insufficient to cause it to burn, letting the molten wax stand in the covered receptacle until most or all of the foamy material accumulated on the top of the wax during the melting is dissolved, pouring the wax into hot molds, and slowly 10 cooling the wax in the molds whereby smooth coherent fine-grained cakes of carnauba wax are produced.

6. A method of preparing smooth coherent fine-grained cakes of carnauba wax which comprises allowing molten carnauba wax to stand and settle in a covered receptacle for about twenty minutes, then pouring the wax into hot molds, and controlling the cooling of the wax in the molds so that it takes from 15 twelve to twenty-four hours, more or less, for the temperature of the wax to drop from slightly above its melting point to substantially room temperature.

7. A method of preparing carnauba wax which comprises melting raw carnauba wax in a covered receptacle by means of an electric heater while keeping the temperature low enough to prevent burning the wax, turning off the heat and letting the molten 20 wax stand in the receptacle until most of the foamy material accumulated on the top of the wax during the melting is dissolved, pouring the wax into hot molds, and cooling the molds of wax sufficiently slowly to cause 25 the cakes of wax to come to room temperature without cracking.

8. A method of preparing carnauba wax which comprises melting raw carnauba wax without permitting the temperature of the wax to rise above about 220° Fahrenheit, separating from the wax whatever dirt may be present, pouring the wax into hot molds, and causing the wax to cool sufficiently slowly so that internal stresses sufficient to 30 make the cakes easily breakable are not set up.

9. A method of preparing carnauba wax which comprises melting raw carnauba wax in a covered receptacle without permitting the temperature of the wax to rise above about 220° Fahrenheit, removing the source 35 of heat and permitting the wax to stand in the covered receptacle about twenty minutes, pouring the wax into hot molds, and pro-

teeting the molds from rapid cooling by suitable insulation so that the cakes of wax are formed without cracks or the occurrence of internal stresses sufficient to cause the cakes to crack or break.

10. A method of preparing carnauba wax which comprises heating raw carnauba wax in a covered receptacle and thereby melting the wax without permitting its temperature to rise above about 220° Fahrenheit, letting the molten wax stand in the covered receptacle without the application of heat until most of the foamy material accumulated on the top of the wax during the melting is dissolved, pouring the wax into hot molds, and slowly cooling the wax in the molds whereby smooth coherent fine-grained cakes of carnauba wax are produced.

11. A method of preparing carnauba wax which comprises melting raw carnauba wax in a covered receptacle by means of an electric heater while keeping the temperature of the wax below about 220° Fahrenheit, turning off the heat and letting the melted wax stand in the receptacle about twenty minutes to permit dirt to settle and the foamy material which rises on the top of the wax during the melting to dissolve, pouring the wax into hot molds, and controlling the cooling of the molds of wax so that the cakes take 40 twelve hours or more to come to room temperature.

12. A method of preparing carnauba wax which comprises melting raw carnauba wax in a covered receptacle at a temperature of about 216° Fahrenheit, permitting the wax to stand in the covered receptacle about twenty minutes with the source of heat removed, pouring the wax into hot molds, and protecting the molds from rapid cooling so that the cakes of wax are formed 45 without cracks or the occurrence of internal stresses sufficient to cause the cakes to crack or break.

13. Unadulterated carnauba wax molded in the form of a coherent fine-grained cake.

14. Unadulterated carnauba wax molded in the form of a coherent cake.

15. Unadulterated carnauba wax in the form of a smooth coherent fine-grained cake.

16. Unadulterated carnauba wax in the form of a smooth coherent cake having a color at least as light as that of the raw wax from which it was prepared.

17. Unadulterated carnauba wax molded in the form of a coherent cake of sufficient strength to stand up without breaking under the treatment which it normally receives in shipment and handling and in being applied to the rotary brushes or pads of polishing machines.

In testimony whereof I have signed my name to this specification.

WILLIAM A. SPRAGUE.